

## UNITED STATES PATENT OFFICE

2,610,911

## METALLURGY

Marvin J. Udy, Niagara Falls, N. Y., assignor to  
 Guaranty Investment Corporation Limited,  
 Montreal, Quebec, Canada, a corporation of  
 Canada

No Drawing. Application September 19, 1945,  
 Serial No. 617,447

4 Claims. (Cl. 75—27)

This invention relates to metallurgy and has for an object the provision of certain improved reaction mixtures for use in metallurgical methods or processes. More particularly, the invention contemplates the provision of certain improved reaction mixtures for use in methods or processes for the production of cast iron. A specific object of the invention is to provide an improved reaction mixture suitable for use in producing high-strength cast iron. A further object of the invention is to provide improved exothermic reaction mixtures suitable for use in the production of high-strength cast iron.

The reaction mixtures of the invention may be employed in any suitable processes, but they are particularly useful for treating cast iron. Cast iron can be treated while in the molten state with an exothermic reaction mixture of the invention comprising silicon, strontium and a nitrate radical to produce cast iron products having improved mechanical or physical properties. Thus, for example, it has been found that by reacting with such a reaction mixture molten cast iron, such as cupola iron and blast furnace iron, containing about two and seventy-five hundredths percent (2.75%) to three and twenty-five hundredths percent (3.25%) of carbon and silicon in amount less than that required for high-strength cast iron, cast iron products having improved transverse, tensile, deflection, impact, hardness and other properties can be produced. The reaction mixtures of the invention are particularly useful in methods or processes for producing gray cast iron. The use of exothermic reaction mixtures of the invention for treating cast iron has little or no effect on the depth of chill.

In carrying out a method or process employing a reaction mixture of the invention, molten cast iron from any suitable source is reacted in a ladle, for example, with an exothermic reaction mixture in amount sufficient to modify the mechanical or physical properties or characteristics of the cast iron by increasing the silicon content without altering substantially the composition of the cast iron with respect to total carbon.

In carrying out a method or process employing a reaction mixture of the invention, I may employ an exothermic reaction mixture comprising a nitrate of any metal of the group consisting of strontium, barium, calcium and magnesium, or I may employ an exothermic reaction mixture comprising a compound of strontium, a nitrate of another metal and silicon. Two or more nitrates may be employed in a reaction mixture if desired. Sodium nitrate may be employed in

conjunction with any one or more of the nitrates of strontium, barium, calcium and magnesium.

Exothermic reaction mixtures of the invention preferably contain ferrosilicon as the source of silicon, and they preferably are formed by grinding together the components to form mixtures of particles most or all of which are small enough to pass a 100-mesh screen. Grinding together of the components results in thorough and intimate mixing which is conducive to effective and complete reaction. The reaction mixtures may be employed in the form of loose powders or in the form of agglomerates or briquets. Any suitable bonding agent may be employed in forming the agglomerates or briquets. When sodium nitrate is employed, it may function as the bonding agent. Thus, for example, a finely divided mixture comprising sodium nitrate may be moistened with water in amount by weight equal to about two to three percent (2 to 3%) of the weight of the mixture, molded, heated to drive off water and melt the sodium nitrate and cooled to permit solidification of the sodium nitrate in place. The solidified sodium nitrate is intimately associated with the other components and functions as the bonding agent.

The components of a reaction mixture of the invention are so proportioned as to provide silicon in excess of the amount which can be oxidized by all of the nitrate and any other reducible compound which may be present. The excess silicon enters the molten cast iron, increasing the silicon concentration and causing a graphitizing effect on the carbon contained therein. Nitrate and silicon for oxidation by the nitrate preferably are employed in amounts such that, by reaction, sufficient heat is generated to melt the excess silicon, so that the excess silicon enters the molten cast iron in the molten state and becomes quickly and thoroughly dispersed therein.

The following examples illustrate reaction mixtures of the invention.

(In the various examples illustrating the reaction mixtures, the proportions of the components are set forth in parts by weight.)

## I

|                                                     |      |
|-----------------------------------------------------|------|
| Ferrosilicon (75% Si)                               | 84   |
| Ferrosilicon (50% Si)                               | 16   |
| Strontium nitrate—Sr(NO <sub>3</sub> ) <sub>2</sub> | 22.5 |
| Sodium nitrate—NaNO <sub>3</sub>                    | 2.5  |
| Sodium silicate                                     | .62  |

## II

|                                                     |      |
|-----------------------------------------------------|------|
| Ferrosilicon (75% Si)                               | 83.4 |
| Strontium nitrate—Sr(NO <sub>3</sub> ) <sub>2</sub> | 16.6 |

Ferrosilicon (75% Si) 81.7  
Strontium nitrate—Sr(NO<sub>3</sub>)<sub>2</sub> 18.3

IV  
Ferrosilicon (75% Si) 80.0 5  
Strontium nitrate—Sr(NO<sub>3</sub>)<sub>2</sub> 18.0  
Silica flour 2.0

V  
Ferrosilicon (75% Si) 82.4 10  
Sodium nitrate—NaNO<sub>3</sub> 5.1  
Strontium nitrate—Sr(NO<sub>3</sub>)<sub>2</sub> 12.5

VI  
Ferrosilicon (75% Si) 80.0  
Barium nitrate—Ba(NO<sub>3</sub>)<sub>2</sub> 20.0 15

VII  
Ferrosilicon (75% Si) 100.0  
Strontium nitrate—Sr(NO<sub>3</sub>)<sub>2</sub> 22.5

VIII  
Ferrosilicon (75% Si) 100.0  
Strontium nitrate—Sr(NO<sub>3</sub>)<sub>2</sub> 22.5  
Sodium nitrate—NaNO<sub>3</sub> 2.5

IX  
Ferrosilicon (58.75% Si) 100.0  
Strontium nitrate—Sr(NO<sub>3</sub>)<sub>2</sub> 22.5  
Sodium nitrate—NaNO<sub>3</sub> 2.5

X  
Ferrosilicon (75% Si) 100.0 30  
Strontium nitrate—Sr(NO<sub>3</sub>)<sub>2</sub> 14.6  
Sodium nitrate—NaNO<sub>3</sub> 2.4

XI  
Ferrosilicon (75% Si) 100.0 35  
Strontium nitrate—Sr(NO<sub>3</sub>)<sub>2</sub> 8.9  
Sodium nitrate—NaNO<sub>3</sub> 2.1

The following examples illustrate results obtained in treating molten cast iron products with exothermic reaction mixtures of the types illustrated above (the exothermic reaction mixtures were added to molten cast iron in hand ladles each containing sixty pounds of cast iron, and the metal was stirred well before test-bar castings were poured). 40

| Mixture<br>Added | Chemical Analysis |                    |                    | Mechanical Properties |                 |         |        |
|------------------|-------------------|--------------------|--------------------|-----------------------|-----------------|---------|--------|
|                  | Per-<br>cent<br>C | Per-<br>cent<br>Mn | Per-<br>cent<br>Si | Trans-<br>verse       | Deflec-<br>tion | Tensile | Impact |
| Example VII      | 2.99              | .78                | 1.62               | 3,870                 | .311            | 51,000  | 51.0   |
| Example VIII     | 3.03              | .82                | 1.26               | 3,560                 | .333            | 50,000  | 60.3   |
| Example IX       | 3.02              | .74                | 1.32               | 3,840                 | .273            | 48,800  | 54.2   |
| Example X        | 3.08              | .83                | 1.11               | 3,510                 | .320            | 53,500  | 56.8   |
| Example XI       | 3.08              | .83                | 1.23               | 3,490                 | .345            | 53,800  | 61.8   |

The base iron used in the tests in which the results set forth above were obtained was a low-silicon (.70 to .80% Si) cupola cast iron normally made according to standard commercial cupola practices. 60

| Mixture<br>Added | Chemical Analysis |                    |                    | Mechanical Properties |                 |         |        |
|------------------|-------------------|--------------------|--------------------|-----------------------|-----------------|---------|--------|
|                  | Per-<br>cent<br>C | Per-<br>cent<br>Mn | Per-<br>cent<br>Si | Trans-<br>verse       | Deflec-<br>tion | Tensile | Impact |
| Example VIII     | 3.08              | .42                | 1.72               | 3,625                 | .363            | 51,750  | 62.9   |
| Example X        | 3.08              | .42                | 1.43               | 3,482                 | .369            | 49,620  | 60.4   |
| Example XI       | 3.08              | .42                | 1.21               | 3,505                 | .346            | 49,510  | 63.0   |
| Example IX       | 3.00              | .67                | 1.52               | 3,738                 | .341            | 49,704  | 65.7   |
| Example J        | 2.96              | .67                | 1.72               | 3,800                 | .346            | 51,900  | 64.8   |

The base iron used was similar to that employed in the tests for which results are set forth in Example XII above.

I claim:

1. A reaction mixture suitable for use in treating molten cast iron which comprises (1) silicon, (2) one or more chemically combined elements of the group consisting of calcium, strontium, barium and magnesium and (3) a chemically combined nitrate radical, components of the reaction mixture being of such compositions and being present in such proportions as to be capable of reacting exothermically upon contact with molten cast iron to decompose the nitrate radical with oxidation of silicon.

2. A reaction mixture suitable for use in treating molten cast iron comprising silicon and calcium nitrate, components of the reaction mixture being of such compositions and being present in such proportions as to be capable of reacting exothermically upon contact with molten cast iron to decompose the calcium nitrate with oxidation of silicon.

3. A reaction mixture suitable for use in treating molten cast iron comprising silicon and barium nitrate, components of the reaction mixture being of such compositions and being present in such proportions as to be capable of reacting exothermically upon contact with molten cast iron to decompose the barium nitrate with oxidation of silicon.

4. A reaction mixture suitable for use in treating molten cast iron comprising silicon and magnesium nitrate, components of the reaction mixture being of such compositions and being present in such proportions as to be capable of reacting exothermically upon contact with molten cast iron to decompose the magnesium nitrate with oxidation of silicon.

MARVIN J. UDY.

#### REFERENCES CITED

The following references are of record in the file of this patent:

#### UNITED STATES PATENTS

| Number    | Name    | Date          |
|-----------|---------|---------------|
| 2,243,783 | Udy     | May 27, 1941  |
| 2,280,872 | Udy     | Apr. 28, 1942 |
| 2,444,354 | Kinnear | June 29, 1948 |